

## UNITED STATES PATENT OFFICE.

ARTHUR ARENT, OF DES MOINES, IOWA, ASSIGNOR TO ARTHUR ARENT LABORATORIES, INC., OF DES MOINES, IOWA, A CORPORATION OF IOWA.

## ART OF PROTECTIVELY TREATING MATERIALS.

1,418,610.

Specification of Letters Patent. Patented June 6, 1922.

No Drawing.

Application filed June 9, 1920. Serial No. 387,733.

*To all whom it may concern:*

Be it known that I, ARTHUR ARENT, a citizen of the United States, residing at Des Moines, in the county of Polk and State of Iowa, have invented certain new and useful Improvements in the Art of Protectively Treating Materials; and I do hereby declare the following to be a full, clear, and exact description of the invention, such as will 10 enable others skilled in the art to which it appertains to make and use the same.

This invention relates to art of protectively treating materials; and it has to do more particularly with the treatment of 15 fibrous or absorbent materials with a solution of antimony chlorid,  $SbCl_3$ , dissolved in benzol, for the purpose of rendering such materials resistant to fire or otherwise preserving and protecting the same, said solution 20 also being novel and constituting a part of the invention.

I have found that in the practice of the invention, good results are obtained if fibrous materials, such as wooden shingles, wood in 25 general, wood pulp, paper pulp, paper in general, wallboard, canvass or cloth generally, wooden posts and piling, or the like, be impregnated with a solution of antimony chlorid in benzol, and the solvent be then 30 allowed to evaporate spontaneously, or be driven off by any suitable drying process. The material thus treated and retaining in its pores antimony chlorid is highly resistant to fire and also resists decay in the case of 35 wooden posts, piling, shingles, or like articles, which may be exposed under some conditions of use to borers such as the teredo, for example, the antimony chlorid thus deposited in the pores of the wood acting as 40 a toxic agent enabling the wood to successfully resist the attacks of these destructive agents. Moreover, since the action of moisture on antimony chlorid results in the formation of insoluble antimony compounds, 45 such as oxychlorids for example, the fire-proofing and toxic agent is not washed out of the wood by weathering or by submersion in water, but on the contrary clings tenaciously to the fiber and therefore constitutes 50 a permanent protective agent.

In carrying out the invention in actual practice I dissolve a suitable amount of antimony trichlorid in benzol and then apply the resultant solution to the materials or 55 articles to be protected in the manner de-

scribed. In a typical example, the antimony trichlorid may be employed in the proportion of 2 pounds to 1 gallon of commercial benzol, consisting largely of the compound benzene  $C_6H_6$ ; this proportion (roughly 60 about 25 per cent of the benzol by weight) being effective to render the wood, cloth, or other material non-inflammable after evaporation of the solvent, in the sense that the material thus treated will merely char upon 65 direct application of a flame thereto, but will not take fire. Larger proportions of antimony trichlorid may be employed up to the saturation point of the benzol, where special circumstances require heavier 70 impregnation of the material to be protected. As stated, the benzol may be allowed to evaporate spontaneously but in practice it is desirable to drive off the solvent by appropriate heating and drying means and to 75 recover the solvent for re-use.

Antimony trichlorid itself is a highly effective fireproofing and toxic or preservative agent; and it is not essential, in the broader aspects of the invention, to treat 80 the articles or materials to be protected further than as already described. However, since exposure of the treated materials to atmospheric moisture eventually results in more or less rapid hydrolyzation of the contained antimony salt anyway, it is often desirable in practice in order to hasten and complete this hydrolyzation to specially treat the impregnated materials, after removal of the solvent, with moisture, either 85 in the form of water or steam, thus converting the antimony salt into an oxysalt or a mixture of oxysalts of varying composition, such basic compounds being insoluble in 90 water and clinging tenaciously to and within the fiber of the material. Benzol being an extremely penetrating hydrocarbon solvent, the antimony trichlorid dissolved therein is carried into the very substance of the materials treated and does not merely 95 coat the outer surfaces of the fibres themselves; so that upon subsequent hydrolyzation, either artificially or by normal exposure, to atmospheric moisture, the insoluble basic compounds are distributed through 100 the substance of the material in a thoroughly effective manner and afford the maximum degree of protection.

Where it is desired also to impart a color or stain to the material to be protected, as 110

in the case of shingles or interior woodwork for example, the desired stain may be incorporated with the described impregnating solution without in any way lessening the 5 desired fire-retarding effect. It is also possible to incorporate in the treating solution rubber, varnish gums, drying oils, etc., where a waterproofing or varnishing effect is also desired; and in such cases especially, it is 10 sometimes advisable to increase the proportion of antimony trichlorid above that mentioned in the specific example given, in order to ensure the requisite degree of non-inflammability in the protected material. 15 Whenever necessary, other solvents for rubber or varnish gums, miscible with benzol, may be incorporated in the treated mixture to ensure satisfactory solution of all the constituents and to maintain the 20 penetrating character of the treating solution. Obviously, where varnish gums or the like constitute a part of the treating mixture, the solution may be used like a varnish to externally coat woodwork or the like as 25 distinguished from impregnation or saturation as ordinarily understood. In such cases also, the antimony trichlorid is protected to a large extent from atmospheric influences and therefore changes much more slowly 30 into basic forms; but in any case it remains in or on the materials or articles treated as a permanent protective agent.

For purposes of illustration, various compositions have been described above as 35 within the present invention, but it is to be

understood that numerous other mixtures, within the language of the appended claims, are also included within the invention. Any well known or suitable method of impregnating the materials to be protected may be 40 employed, the invention not being dependent upon the use of any particular mechanical procedure in this respect.

What I claim is:

1. The process of protectively treating materials which comprises applying thereto a solution comprising benzol and antimony trichlorid dissolved therein. 45
2. The process of protectively treating materials which comprises applying thereto a solution comprising benzol, dissolved antimony trichlorid and a waterproofing agent. 50
3. The process of treating wood which comprises impregnating the same with a solution comprising benzol and antimony trichlorid dissolved therein. 55
4. A composition for protectively treating materials which comprises a solution of antimony chlorid in benzol. 60
5. A solution of antimony trichlorid in benzol in the proportion of at least about two pounds of antimony trichlorid to one gallon of benzol. 65
6. A composition for protectively treating materials which comprises a solution of antimony trichlorid and coloring matter in benzol.

In testimony whereof I hereunto affix my signature.

ARTHUR ARENT.